

Patented Mar. 18, 1924.

1,487,136

# UNITED STATES PATENT OFFICE.

HARRY H. ALEXANDER, OF WESTFIELD, NEW JERSEY, ASSIGNOR TO AMERICAN SMELTING AND REFINING COMPANY, OF NEW YORK, N. Y., A CORPORATION OF NEW JERSEY.

## ELECTROLYTIC REFINING OF TIN.

No Drawing. Application filed December 30, 1920, Serial No. 434,124. Renewed October 26, 1923.

To all whom it may concern:

Be it known that I, HARRY H. ALEXANDER, a citizen of the United States, and resident of Westfield, in the county of Union and 5 State of New Jersey, have invented certain new and useful Improvements in Electrolytic Refining of Tin, of which the following is a specification.

The invention relates to certain new and 10 useful improvements in the production of an electrolytically refined tin from impure tin anodes and the present disclosure constitutes an improvement over the disclosure in the patent to R. L. Whitehead, #1,157-, 15 830, October 26, 1915.

It is suggested in this patent that in the electrolytic refining of tin containing lead, an amount of sulphuric acid be added to the electrolyte, which contains metallic tin dissolved in hydrofluosilicic acid, in an amount sufficient to convert the lead present into lead sulfate which is insoluble in the electrolyte. The patentee suggests the employment in a twenty-per cent solution of hydrofluosilicic acid to insure the continued maintenance of the electrolytic decomposition of the tin during the refining operation.

Under some conditions this electrolyte did not prove entirely satisfactory especially 30 when an addition agent, such as glue was added. For instance, polarization would occur, necessitating the frequent removal of the cathode plates, silica ( $SiO_2$ ) would deposit on the anodes and when attempts were 35 made to heat this electrolyte as suggested in the application of Stack Serial No. 434,114, filed under even date there would result a loss of acid as silicon fluoride ( $SiF_4$ ). It was a usual practice in using the patented electrolyte to line the tanks with tar paper and pitch which rapidly deteriorated especially 40 when cresylic acid was used as one of the addition agents in the manner suggested in the application of Frank C. Mathers, Serial 45 No. 257,700, filed October 11, 1918.

The primary object of the present invention is to provide an electrolyte which will effectively and continuously dissolve the tin, which will precipitate the lead from the anode, which will prevent the formation of the basic salts of tin, will render the anode entirely soluble, prevent polarization and permit the use of a tank lining which will be substantially unaffected by the contents of 50 the tank.

Incidentally other objects of the invention is to attain high current efficiency and to obtain a smooth, dense, adherent deposit of tin of high purity.

I attain this invention broadly simply by 60 changing the character of the electrolyte defined in the Whitehead patent, above identified, from a hydrofluosilicic acid basis to a sulphuric acid basis. Instead of using merely sufficient sulphuric acid to unite with 65 the lead present in the electrolyte a materially excessive amount of sulphuric acid is used. Further and mainly for the purpose of featuring economy in the use of the relatively expensive hydrofluosilicic acid, 70 the contents of this acid in the electrolyte is reduced with beneficial effect. While it is within the scope of this disclosure to suggest any amount of sulphuric acid in excess of the amount necessary to precipitate the 75 lead it has been found in practice that six to eight per cent of free sulphuric acid gives the best conductivity and anode corrosion, but this proportion is only suggestive of one situation in which it was found satisfactory. 80

Certain additional agents such as cresylic acid and glue or cresol sulphonic acid, as suggested in the above identified Stack application, were used with a resulting improvement in the character of the deposits. 85

In operation the electrolytic tanks are arranged preferably in batteries with the impure tin usually cast in anodes and each operatively associated in a lead lined tank 90 with a cathode usually formed of tin. A direct current of suitable voltage and of about eight amperes per square foot of cathode surface is passed from the impure tin as anodes to the cathodes through the 95 sulphuric hydrofluosilicic acid electrolyte as is well known in the practicing of such processes. The tin is dissolved from the anodes into the electrolyte and deposited out of the electrolyte upon the cathode plates. 100 The impurities usually found in such tin will not dissolve from the anode in the presence of the large excess of tin present and the lead which dissolves is precipitated as sulfate and appears as a slime which is 105 later subjected to other treatments in order to retain its values.

With this sulphuric acid electrolyte it was possible to use lead lined tanks without danger of destruction from the electrolyte. 110

The presence of the large excess of sulphuric acid prevents any solvent action of the sulphurous acid on the lead and the presence of the hydrofluosilicic acid even in the reduced proportions herein suggested prevented the formation of basic salts of tin, rendered the anode soluble and prevented polarization.

Having thus described my invention, I claim:

10. 1. In the electrolytic refining of impure tin containing lead, the method of refining tin which consists in passing an electric current of suitable voltage and amperage from the impure tin as an anode to a cathode through an electrolyte which is a solvent of tin and lead and protecting the electrolyte from contamination by lead, by incorporating with the electrolyte an agent which will combine with the lead to form an insoluble compound, said agent being present in an amount materially in excess of the amount necessary to unite with all the lead present in the electrolyte.
15. 2. In the electrolytic refining of impure tin containing lead, the method of refining tin which consists in passing an electrolytic current of suitable voltage and amperage from the impure tin as an anode to a cathode through a solution of hydrofluosilicic acid containing an amount of sulphuric acid greatly in excess of the amount sufficient to combine with the lead in the electrolyte to form lead sulphate.
20. 3. In the electrolytic refining of impure tin, the method of preventing contamination of the tin deposited from the impure tin anode upon the cathode, which consists in employing as the electrolyte a solution of tin in hydrofluosilicic acid together with a quantity of sulphuric acid in excess of the amount sufficient to convert the lead of the dissolving anode into lead sulphate thereby to leave some free sulphuric acid in the electrolyte.
25. 4. The process for the refining of impure tin, which comprises passing an electrolytic current of suitable voltage and amperage

from a tin anode to a cathode through a solution of hydrofluosilicic acid contained in a lead lined tank and adding to the solution an agent which will protect the tank lining from the solvent action of the hydrofluosilicic acid.

5. An electrolyte for the deposition of tin free from lead, comprising an electrolytic solution of tin in hydrofluosilicic acid containing a large amount of sulphuric acid, whereby, upon the passage of a current therethrough from an impure tin anode containing lead to a cathode, the tin will be dissolved from the anode and deposited on the cathode without contamination with lead and in the presence of an excess of the sulphuric acid.

6. In the electrolytic refining of impure tin containing lead, the method of refining tin which consists in passing an electrolytic current of suitable voltage and amperage from the impure tin as an anode to a cathode through a solution of hydrofluosilicic acid three to five per cent and free sulphuric acid six to eight per cent.

7. In the electrolytic refining of impure tin containing lead, the method of refining tin which consists in passing an electrolytic current of suitable voltage and amperage from the impure tin as an anode to a cathode through a solution of hydrofluosilicic acid three to five per cent and free sulphuric acid six to eight per cent and in the presence of an addition agent.

8. In the electrolytic refining of impure tin containing lead, the method of refining tin which consists in passing an electrolytic current of suitable voltage and amperage from the impure tin as an anode to a cathode through a solution of hydrofluosilicic acid three to five per cent and free sulphuric acid six to eight per cent and in the presence of cresylic acid and glue.

Signed at Maurer, in the county of Middlesex and State of New Jersey this twenty-second day of December, A. D. 1920.

HARRY H. ALEXANDER.